

Dec. 13, 1927.

1,652,556

P. H. BRACE

BIMETALLIC THERMOSTAT MATERIAL

Filed March 12, 1925



WITNESSES:

R. J. Fitzgerald  
N. M. Biebel

INVENTOR

Porter H. Brace

BY

Wesley L. Barr

ATTORNEY

Patented Dec. 13, 1927.

1,652,556

# UNITED STATES PATENT OFFICE.

PORTER H. BRACE, OF WILKINSBURG, PENNSYLVANIA, ASSIGNOR TO WESTINGHOUSE ELECTRIC & MANUFACTURING COMPANY, A CORPORATION OF PENNSYLVANIA.

## BIMETALLIC THERMOSTAT MATERIAL.

Application filed March 12, 1925. Serial No. 14,970.

My invention relates to temperature controlled devices and particularly to bimetallic thermostats.

One object of my invention is to provide a bimetallic thermostat, the elements of which shall have a relatively large difference between their respective temperature coefficients of expansion, and that shall be composed of material capable of being subjected 10 to relatively high temperatures without deterioration in its operating characteristics.

Another object of my invention is to provide a bimetallic thermostat comprising two closely related alloys that shall however, 15 have dissimilar temperature coefficients of expansion.

Another object of my invention is to provide a bimetallic thermostat comprising two closely related alloys, the composition of 20 one or both of which may be varied in accordance with the desired temperature limits within which the said device is to operate.

In practicing my invention, I provide a bimetallic thermostat that is made up of an 25 irreversible and a reversible nickel steel. The amount of nickel in the reversible nickel steel varies substantially in accordance with the upper temperature limit within which it is desired that the thermostat shall operate.

30 In the single sheet of drawings, I have illustrated temperature-expansivity curves of alloys of nickel steel containing different percentages of nickel, which alloys I employ in making bimetallic thermostats.

35 The numeral 11 designates a curve of thermal temperature coefficient of a nickel steel alloy containing or comprising substantially 26% of nickel. This curve is substantially a straight line between the limits 40 of zero and of 500° C. and it may be noted that the value of the temperature coefficients of expansion increase with an increase in the temperature.

A nickel steel alloy containing substantially 45 26% of nickel is an alloy that is within the range of composition covered by the so-called irreversible nickel steels. However, the expansion of such a nickel steel is reversible between certain temperature 50 limits, which limits are dependent upon the nickel content, provided the material has been heat treated at a temperature above its transformation point. For 26% nickel steel the limit is approximately -20° C. at the 55 lower end of the scale and above 600° C. to

650° C. at the upper end of the scale, a temperature at which the elastic limit of the metal is still high enough to permit of its use in bimetallic elements.

Hence, a material or alloy having this 60 percentage of nickel may be employed in a bimetallic or thermostatic device provided that it has been properly heat treated, and further, that the minimum temperature to which it is subjected in actual operation does 65 not fall below substantially -20° C. and does not rise above substantially 600 to 650° C. If the device is operated within these limits, the temperature coefficients of expansion 70 will be substantially those indicated by the curve designated by the numeral 11. The lower temperature limit may be varied by varying the percentage of nickel in the alloy, and it may be materially reduced below the 75 figure above given by increasing the percentage of nickel in the alloy.

The heat treatment of the irreversible nickel steels consists in heating them to a temperature above the A<sup>2</sup> transformation point. In pure iron this occurs at a temperature in the neighborhood of 900° C. This transformation point is progressively lowered by increasing quantities of nickel and the temperature at which it occurs on heating becomes more and more widely separated from the temperature at which it occurs on cooling. It is this temperature-hysteresis of the thermal effect which gives rise to the appellation "irreversible". For nickel contents above approximately 30% 80 the transformation disappears and the length-temperature curves on heating coincide very closely with those on cooling, hence these alloys are called reversible alloys. If an irreversible alloy is heated above its 85 upper transformation point and not subsequently cooled below its lower transformation point, it will expand and contract in a nearly reversible manner but at a much higher rate than normal. It is this property 90 of the irreversible nickel steels that is taken advantage of in order to obtain relatively high and reversible thermal expansivity.

100 The second element of my heat responsive device comprises a nickel steel alloy having a different amount of nickel, and in general the percentage of nickel in the second element will exceed 30% and the numeral 12 indicates a curve illustrating the temperature coefficient of expansion of a nickel steel 105 110

alloy having approximately 42% nickel. This material is within the range of compositions covered by the so-called "reversible" nickel steels, and it may be noted further that the temperature coefficient of expansion of the 42% nickel steel approaches that of the 26% nickel steel when the material is subjected to a temperature substantially in excess of 300° C. The curve of temperature coefficients of expansion up to 300° C. indicates that the values thereof decrease somewhat with increased temperatures up to 300° C. and are different than those possessed by the 26% nickel steel.

15 As indicated by the curves 11 and 12, the temperature coefficient of expansion of the 26% nickel steel is substantially three times that of the 42% nickel steel for temperatures between zero and substantially 20 300° C. Hence, it is obvious that a heat-responsive device made in the form of a bimetallic thermostat in which two bars one of 26% and the other of 42% nickel steel are suitably fixedly connected at their ends 25 or are connected over their entire abutting faces or surfaces, as by welding, will have relatively large deflections for given changes of temperature when the heat-responsive device is mounted and employed in the usual 30 manner well known in the art.

A heat-responsive device comprising a 26% and a 42% nickel steel will, therefore, be operative for a temperature range of substantially zero to 300° C.

35 If it is desired to increase this temperature range, particularly at the upper limit thereof, I may employ a nickel steel for one of the elements that has a relatively higher percentage of nickel. The temperature coefficients of expansion of a 57% nickel steel are indicated in the curve designated by the numeral 13. The temperature coefficients of expansion are relatively greater than those for the 42% nickel steel 40 at the lower temperatures but are lower at temperatures substantially above 350° C. The values of the coefficients are also less subject to variation and a heat-responsive device embodying metallic elements comprising alloys having 26 and 57% respectively of nickel may be employed at temperatures up to approximately 500° C.

55 While the nickel steel alloy for 57% nickel is irreversible, the transformation points occur at temperatures beyond 500° or even 550° C. and hence a heat-responsive device comprising these metallic elements will operate satisfactorily within the temperature range of 0° C. to within 500° C.

60 As it is important to retain a relatively high elastic limit of the metallic elements at the high temperatures to which they will be subjected, I may incorporate other metals in the respective alloys. I may use, for in-

stance, cobalt, chromium, tungsten, molybdenum, silicon, aluminum, manganese, tantalum or vanadium or suitable combinations thereof. In general, the percentage of such auxiliary elements will not exceed 15% and will usually be below this value. The addition of one or several of the above metals, in amounts of not to exceed 15% modifies the position of the transformation points and hence the temperature range over which the device can be used, the shape of the expansivity-temperature curves, and, most important of all, increases the elastic limit of the material at the higher temperatures.

The device embodying my invention thus comprises a plurality of metallic elements 30 that are combined or connected in order that their respective temperature coefficients of expansion may cause a deflection of one part of the device relatively to the other part, in a manner well known in the art. 35 The metallic elements are closely related in that they comprise nickel steel alloys of different nickel content, the percentage of nickel being increased in accordance with the maximum temperature at which it is 40 desired that the heat-responsive device shall operate properly. Auxiliary metals, in relatively small percentages, may be added, to increase the elastic limit of the 45 alloys at the higher temperatures. 95

Various modifications and changes may be made without departing from the spirit and scope of the invention, I desire, therefore, that only such limitation shall be placed thereon as are imposed by the prior 100 art.

I claim as my invention:

1. A heat-responsive device consisting of two metallic elements of nickel steel alloys, the nickel to iron ratio in one of said elements being less than .3 and being more than .3 in the other element. 105

2. A heat-responsive device comprising two metallic elements each consisting of a nickel steel alloy, the nickel to steel ratio in one of said elements being less than .3 and being more than .3 in the other element, and both elements containing less than 15% of metals tending to increase the elastic limit of the elements at temperatures above 110 300° C. 115

3. A heat-responsive device comprising a bimetallic structure, each element of which is a nickel steel alloy and such percentages of other metals to so change the transformation points of the component nickel steel alloys as to permit them to be employed over any desired temperature ranges. 120

In testimony whereof, I have hereunto subscribed my name this 9th day of March, 125 1925.

PORTER H. BRACE.